# EUROPEAN PATENT SPECIFICATION

(11) **EP 2 095 895 B1**
(45) Date of publication and mention of the grant of the patent: **06.03.2013**
(21) Application number: 07828677.0
(22) Date of filing: 28.09.2007
(51) Int. Cl.: B22D 17/00, B22C 9/10, B22D 17/22, B22D 17/32, C22F 1/00, C22F 1/04

(54) **ALUMINUM DIE CAST PRODUCT AND PROCESS FOR MANUFACTURING THE SAME**
ALUMINIUMDRUCKGUSSPRODUKT UND VERFAHREN ZU DESSEN HERSTELLUNG
PRODUIT EN ALUMINIUM COULÉ SOUS PRESSION ET PROCÉDÉ DE FABRICATION DE CELUI-CI

(30) Priority: 20.12.2006 JP 2006342909
(43) Date of publication of application: 02.09.2009
(73) Proprietor: Mitsubishi Heavy Industries, Ltd., Tokyo 108-8215 (JP)
(72) Inventor: HAMASAKI, Masafumi, Nagoya-shi Aichi 453-8515 (JP); INOGUCHI, Kazuhiko, Nagoya-shi Aichi 453-8515 (JP); HATANAKA, Masaya, Nagoya-shi Aichi 453-8515 (JP); KAWASAKI, Masaki, Kiyosu-shi Aichi 452-8561 (JP); SAHO, Shinji, Higashiosaka-shi Osaka 577-0835 (JP)
(74) Representative: Besnard, Christophe Laurent
(86) International application number: PCT/JP2007/068935
(87) International publication number: WO 2008/075491

(56) References cited:
- EP-A2- 1 557 567
- JP-A- 09 277 014
- JP-A- 2004 225 134
- JP-A- 2004 330 273

## Description

### Technical Field

The present invention relates to an aluminum die cast product that can be advantageously used, e.g., for a pressure container that requires high airtightness, as in a compressor housing, and to a method for manufacturing the aluminum die cast product.

### Background Art

A solidification shrinkage space is known to occur in aluminum die cast products as a result of solidification shrinkage of a melt injected into a die during die cast molding. In the case of aluminum alloys, a volume shrinkage of about 6% occurs during solidification. Shrinkage cavities occur due to inclusion of such shrinkage spaces in the product, and the shrinkage cavities become casting defects. Shrinkage cavities tend to expand to a wide range where the cast portion has a large thickness or a low cooling rate.
In die cast products, the cooling rate of a portion located close to the surface (casting surface) that is in contact with a die is generally high and, therefore, a region with a small number of defects that is called a chill layer is formed at the casting surface. However, because the cooling rate is low inside thick portions, shrinkage cavities occurring due to solidification shrinkage are formed therein. In most cases, the shrinkage cavities are formed via three-dimensional expansion.

For example, in the case of a compressor housing, which is a pressure container, a port hole for taking in and discharging a cooling gas and a screw hole for attaching a fitting serving to connect a pipe to the port hole are provided in a thick portion that is thicker than other portions of the housing. Cast holes obtained by die casting using core pins usually serve as rough holes for the port hole and screw hole, and because the dimensional accuracy of as-cast products is low, machining is typically performed with a cutting allowance of about 0.5 mm.
In this case, although no defects are present on the casting surface and the appearance is beautiful, the shrinkage cavity defects sometimes appear inside, as described hereinabove. As a result, where the thickness of the region without shrinkage cavity defects is less than the cutting allowance, the shrinkage cavity defects are exposed on the cut surface after the cutting, thereby creating a risk of causing the inside and outside of the housing, or the port hole and screw hole to be linked to each other. This can cause pressure leak or cooling gas leak and becomes an important reason for the decrease in the product yield.

On the other hand, a local pressurization method and a local cooling method (see, for example, Patent Citation 1) are known as methods for inhibiting the occurrence of shrinkage cavity defects in the thick portions, and it has been empirically established that the occurrence of shrinkage cavity defects can be inhibited by intensifying local cooling.
Further, a core pin for die casting a cast hole has been suggested (see, for example, Patent Citation 2), the pin having a configuration in which a cooling water path is formed by fitting a cooling water pipe into the core pin body and cooling water is forced to flow in the cooling water path. Furthermore, a process of casting a rough hole for a bolt hole provided in a cylinder block has been described as an example.

Patent Citation 1: Japanese Unexamined Patent Application, Publication No. 2004-223610.
Patent Citation 2: Japanese Unexamined Patent Application, Publication No. Hei 9-323149.

### Disclosure of Invention

As described above, the effectiveness of local cooling intensification in inhibiting the occurrence of shrinkage cavity defects has been recognized by those skilled in the art.
However, it is presently not clear how to the cooling should be intensified to inhibit the occurrence of shrinkage cavity defects, to what degree a region without shrinkage cavity defects is formed due to intensification of cooling, what correlation exists between the intensification of cooling and the growth of dendrites during solidification shrinkage of the melt, and whether the shrinkage cavity defects causing pressure leak or gas leak do not occur if the growth of dendrites is somehow controlled. There is thus a need for establishing a technology that can reduce a pressure leak or gas leak ratio and increase the product yield in the manufacture, e.g., of pressure containers that require a high degree of airtightness, as in compressor housings.

The present invention was created in view of the foregoing, and it is an object of the present invention to provide an aluminum die cast product, e.g., a pressure vessel that requires high airtightness, in which pressure leak or gas leak ratio can be reduced and in which the product yield can be increased, and also to provide a method for manufacturing the product.

The aluminum die cast product and method for the manufacturing the same in accordance with the present invention utilize the following means to resolve the above-described problems.
Thus, the aluminum die cast product in accordance with the present invention is an aluminum die cast product in which a cast hole is formed by a core pin in a thick portion that is made thicker than other portions, wherein a chill layer with a secondary dendrite arm spacing of at least 5.5 µm or less is provided at the surface of the cast hole.

The tests conducted by the inventors have demonstrated that the growth of dendrites during solidification shrinkage of a melt is inhibited by the intensification of local cooling, and where the secondary dendrite arm spacing is at least 5.5 µm or less, a chill layer can be formed in which shrinkage cavity defects that cause pressure leak or gas leak do not appear on the casting surface. In accordance with the present invention, a chill layer with a secondary dendrite arm spacing of at least 5.5 µm or less is provided at the surface of cast holes in the aluminum die cast product in which cast holes are formed by core pins. Therefore, where the cast holes serve as rough holes, the shrinkage cavity defects are not exposed on the surface thereof and the occurrence of pressure leak or gas leak via the cast holes can be reliably inhibited. Therefore, when a pressure vessel or the like is manufactured, the yield thereof can be greatly increased.
The secondary dendrite arm spacing is a distance between the centers of the adjacent secondary dendrite arms and it is represented by an average value of secondary dendrite arm spacing in a portion where four or more secondary dendrite arms are continuously arranged side by side. More specifically, a portion in which four or more secondary dendrite arms are arranged side by side is selected, a total of n (n is 4 or more) spacings 1 of secondary dendrite arm spacings are measured, and 1/(n - 1) is found. The measurements are performed in three or more locations and an arithmetical average of the results is found.

Further, the aluminum die cast product in accordance with the present invention is the above-described aluminum die cast product in which a thickness of a chill layer with a secondary dendrite arm spacing of at least 5.5 µm or less is made larger than a cutting allowance of the cast hole that is set in advance.

In accordance with the present invention, the thickness of the chill layer with a secondary dendrite arm spacing of at least 5.5 µm or less is made larger than a cutting allowance of the cast hole that is set in advance. Therefore, even when the cast hole is machined as a rough hole by cutting, the machining surface thereof can be confined within a range of the chill layer with a secondary dendrite arm spacing of at least 5.5 µm or less in which the shrinkage cavity defects have not occurred. Therefore, the shrinkage cavity defects are not exposed on the cutting surface, and the occurrence of pressure leak or gas leak directly from the cast hole portion or via a screw hole, or the like, adjacent to the cast hole portion can be reliably inhibited.

Further, the aluminum die cast product in accordance with the present invention is the above-described aluminum die cast product in which the chill layer with a secondary dendrite arm spacing of at least 5.5 µm or less remains after cutting has been performed with the aforementioned cutting allowance.

In accordance with the present invention, because the chill layer with a secondary dendrite arm spacing of at least 5.5 µm or less remains after cutting has been performed with the cutting allowance, the chill layer in which no shrinkage cavity defects have occurred remains at the cast hole surface in the product after cutting. Therefore, the exposure of shrinkage cavity defects on the cutting surface can be reliably prevented and the occurrence of pressure leak or gas leak directly from the cast hole portion or via a screw hole, or the like, adjacent to the cast hole portion can be reliably inhibited.

Further, the aluminum die cast product in accordance with the present invention is any of the above-described aluminum die cast products in which the thickness of the chill layer with a secondary dendrite arm spacing of at least 5.5 µm or less is at least 0.5 mm or more.

In accordance with the present invention, because the thickness of the chill layer with a secondary dendrite arm spacing of at least 5.5 µm or less is at least 0.5 mm or more, the thickness of the chill layer with a secondary dendrite arm spacing of at least 5.5 µm or less can be made larger than the cutting allowance of aluminum die cast products that is generally set to 0.5 mm or less. As a result, the chill layer in which no shrinkage cavity defects have occurred can be reliably left at the surface of cast hole after cutting. Therefore, the shrinkage cavity defects are not exposed on the cutting surface and the occurrence of pressure leak or gas leak directly from the cast hole portion or via a screw hole, or the like, adjacent to the cast hole portion can be reliably inhibited.

Further, the aluminum die cast product in accordance with the present invention is any of the above-described aluminum die cast products in which the aluminum die cast product is a pressure vessel.

In accordance with the present invention, because the aluminum die cast product is a pressure vessel, a pressure vessel can be obtained in which no internal fluid leak occurs from the cast hole via the shrinkage cavity defects. Therefore, when an aluminum die cast pressure vessel is manufactured, the yield thereof can be greatly increased and a high-quality pressure vessel can be obtained at a low cost.

Further, the aluminum die cast product in accordance with the present invention is the above-described aluminum die cast product in which the pressure vessel is a compressor housing.

In accordance with the present invention, because the pressure vessel is a compressor housing, it is possible to obtain a compressor housing with high airtightness in which no internal cooling gas leaks from the cast hole via the shrinkage cavity defects. Therefore, when an aluminum die cast compressor housing is manufactured, the yield thereof can be greatly increased and a high-quality compressor housing can be obtained at a low cost.

The method for manufacturing an aluminum die cast product in accordance with the present invention is a method for manufacturing an aluminum die cast product in which a cast hole is formed by a core pin in a thick portion that is made thicker than other portions, wherein a chill layer with a secondary dendrite arm spacing of at least 5.5 µm or less is formed to a thickness equal to, or larger than a predetermined thickness at the cast hole surface by passing a flow of a cooling medium through the core pin and locally cooling the cast hole.

In accordance with the present invention, by passing a flow of a cooling medium through the core pin and increasing the local cooling capacity with the core pin during die casting, the temperature gradient during melt solidification shrinkage can be increased. Therefore, the growth of dendrites can be inhibited and the chill layer with a secondary dendrite arm spacing of at least 5.5 µm or less can be formed to a thickness equal to, or larger than a predetermined thickness at the cast hole surface. As a result, no shrinkage cavity defects are exposed on the surface of the cast hole even when it is used as a rough hole, the occurrence of pressure leak or gas leak via the cast hole can be reliably inhibited, and a yield in the manufacture of aluminum die cast products such as pressure vessels can be greatly increased.

Further, the method for manufacturing an aluminum die cast product in accordance with the present invention is the above-described method for manufacturing an aluminum die cast product in which a core pin with a double-pipe structure in which a central pipe is inserted into a hollow core pin body is used as the core pin, the cooling medium is supplied from the central pipe to a distal end portion of the core pin, the cooling medium is forced to flow into a cooling medium channel between the central pipe and the pin body, and the cast hole is locally cooled.

In accordance with the present invention, because a core pin with a double-pipe structure in which a central pipe is inserted into a hollow core pin body is used as the core pin, the cooling medium is supplied from the central pipe to a distal end portion of the core pin, and the cooling medium is forced to flow into a cooling medium channel between the central pipe and the pin body, a uniform cooling medium flow channel is formed along the entire periphery, the flow rate of the cooling medium can be stabilized, and local cooling of the cast hole can be performed uniformly. As a result, the chill layer with a secondary dendrite arm spacing of at least 5.5 µm or less can be reliably formed to a thickness equal to, or larger than a predetermined thickness at the cast hole surface with uniformity over the entire periphery. Therefore, the quality of the aluminum die cast product obtained by casting can be stabilized and the yield thereof can be increased.

Further, the method for manufacturing an aluminum die cast product in accordance with the present invention is the above-described method for manufacturing an aluminum die cast product, wherein the cooling medium is caused to flow at a flow rate of 12 cc/s or more.

In accordance with the present invention, because the cooling medium is caused to flow at a flow rate of 12 cc/s or more, the temperature gradient during melt solidification shrinkage is sufficiently increased and the dendrite growth is inhibited. As a result, the chill layer with a secondary dendrite arm spacing of at least 5.5 µm or less can be reliably formed to a thickness equal to, or larger than a predetermined thickness at the cast hole surface.

Further, the method for manufacturing an aluminum die cast product in accordance with the present invention is the above-described method for manufacturing an aluminum die cast product, wherein a core pin of a partition plate structure in which a partition plate arranged along a pin axial direction is inserted into a hollow core pin body is used as the core pin, the cooling medium is supplied from one of the cooling medium channels partitioned by the partition plate, the cooling medium is caused to flow into the other cooling medium channel, and the cast hole is locally cooled.

In accordance with the present invention, because a core pin of a partition plate structure in which a partition plate arranged along a pin axial direction is inserted into a hollow core pin body is used as the core pin, the cooling medium is supplied from one of the cooling medium channels partitioned by the partition plate, and the cooling medium is caused to flow into the other cooling medium channel, a uniform cooling medium flow channel can be formed, the flow rate of the cooling medium can be stabilized, and the cooling performance can be improved. As a result, the chill layer with a secondary dendrite arm spacing of at least 5.5 µm or less can be reliably formed to a thickness equal to, or larger than a predetermined thickness at the cast hole surface. Therefore, the quality of the aluminum die cast product obtained by casting can be stabilized and the yield thereof can be increased.

Further, the method for manufacturing an aluminum die cast product in accordance with the present invention is any of the above-described methods for manufacturing an aluminum die cast product, wherein the flow of the cooling medium is initiated simultaneously with, or immediately prior to the completion of melt injection.

In accordance with the present invention, because the flow of the cooling medium is initiated simultaneously with, or immediately prior to the completion of melt injection, no adverse effect, such as melt overcooling and melt flow disruption, is produced on melt injection, and rapid cooling can be performed simultaneously with completion of injection. As a result, the temperature gradient during melt solidification shrinkage can be sufficiently increased and dendrite growth can be inhibited. Therefore, the chill layer with a secondary dendrite arm spacing of at least 5.5 µm or less can be reliably formed to a thickness equal to, or larger than a predetermined thickness at the cast hole surface.

With the aluminum die cast product and method for manufacturing the same in accordance with the present invention, the chill layer with a secondary dendrite arm spacing of at least 5.5 µm or less can be reliably formed to a thickness equal to, or larger than a predetermined thickness at the cast hole surface. As a result, where the cast hole serves as a rough hole, the shrinkage cavity defects are not exposed on the surface thereof and the occurrence of pressure leak or gas leak via the cast hole can be reliably inhibited. Therefore, when a pressure vessel or the like is manufactured, the yield thereof can be greatly increased and high-quality aluminum die cast products can be manufactured at a low cost.

### Brief Description of Drawings

[FIG. 1] FIG. 1 is a perspective view illustrating the external appearance of a compressor housing that is an aluminum die cast product of one embodiment of the present invention.
[FIG. 2] FIG. 2 is a cross-sectional view along arrows Y-Y of the compressor housing shown in FIG. 1.
[FIG. 3] FIG. 3 is a partial simplified cross-sectional view illustrating a die casting state of the compressor housing shown in FIG. 1.
[FIG. 4] FIG. 4 is a cross-sectional view illustrating an example of a core pin employed for die casting of the compressor housing shown in FIG. 1.
[FIG. 5] FIG. 5 is a cross-sectional view illustrating another example of a core pin employed for die casting of the compressor housing shown in FIG. 1.
[FIG. 6] FIG. 6 is a conceptual diagram illustrating solidification shrinkage of the melt in the case of a small temperature gradient during die cooling.
[FIG. 7] FIG. 7 is a conceptual diagram illustrating solidification shrinkage of the melt in the case of a large temperature gradient during die cooling.
[FIG. 8] FIG. 8 illustrates observations performed with an optical microscope for DAS measurements.
[FIG. 9] FIG. 9 is a graph illustrating the relationship between a cooling water flow rate V (cc/s) and a thickness t (mm) of the region free of shrinkage cavity defects.
[FIG. 10] FIG. 10 is a graph illustrating the relationship between a depth d (mm) from the casting surface in which shrinkage cavity is observed and DAS (µm).

### Explanation of Reference:

1: compressor housing
2: port hole
2A: cast hole
2B: chill layer
4: thick portion
5, 50: core pin
5A: pin body
5E: central pipe
5F, 50I, 50J: cooling medium channel
50E: partition plate
20: dendrite arm
21: secondary dendrite arm
DAS: secondary dendrite arm spacing

### Best Mode for Carrying Out the Invention

An embodiment of the present invention will be described below with reference to the drawings.
FIG. 1 is a perspective view of a compressor housing 1 of one embodiment of the present invention. FIG. 2 is a cross-sectional view along arrows Y-Y in FIG. 1. In the present embodiment, the compressor housing 1, which is a pressure vessel requiring airtightness, is explained as an example of an aluminum die cast product, but the aluminum die cast product in accordance with the present invention is not limited thereto.

The compressor housing 1 constitutes the outer shell of the compressor, and a compression mechanism (not shown in the figure) is contained inside thereof. The compression mechanism compresses a low-pressure cooling gas sucked in via a port hole 2 from the outside of the compression housing 1 and discharges the resultant high-pressure cooling gas to the outside via a port hole (not shown in the figure) provided in the compression housing 1. The compression housing 1 forms a compressor accommodation space that covers and seals the outer periphery of the compression mechanism so as to prevent leak to the outside as the cooling gas is taken in, compressed, and discharged, and the compression housing acts as a pressure vessel.

The aforementioned port hole 2 is provided so as to pass through the compression housing 1, as shown in FIG. 2, and a cooling medium pipe (not shown in the figure) is connected to the port hole 2.
A thick portion 4 that is thicker than other portions is provided in the outer peripheral portion of the compression housing 1, and the port hole 2 is provided together with a screw hole 3 for attaching a fitting for connecting the cooling medium pipe in this thick portion 4. However, the screw hole 3 is not necessarily provided and may be omitted.
The compression housing 1 is produced from an aluminum alloy in order to reduce weight and is manufactured by die casting. The rough holes of the port hole 2 and screw hole 3 are formed as cast holes 2A and 3A with core pins during die casting and then finished by machining to predetermined dimensions after die casting.

FIG. 3 is a schematic sectional view illustrating a state in which the cast holes 2A and 3A for the port hole 2 and screw hole 3 are die cast with core pins 5 and 6. A molding space 9 of the thick portion 4 for molding the cast holes 2A and 3A is formed by a fixed die 7 and a movable die 8. The core pins 5 and 6 for molding the cast holes 2A and 3A are introduced from the side of the fixed die 7 into the molding space 9 and disposed therein. During die casting, the molding space 9 is filled with a melt, thereby molding the cast holes 2A and 3A serving as rough holes for the port hole and screw hole 3 with the core pins 5 and 6.

The thick portion 4 where the port hole 2 and screw hole 3 are provided is thicker than other portions, and during die casting, a solidification shrinkage space is produced by solidification shrinkage of the melt and shrinkage cavity defects easily appear therein. As described above, because the cast holes 2A and 3A molded by the core pins 5 and 6 are finished to obtain the port hole 2 and screw hole 3, where a chill layer 2B on the casting surface is cut, the shrinkage cavity defects can be exposed on the cutting surface and the inside and outside of the compressor housing 1 or the port hole 2 and screw hole 3 can be lined together via the shrinkage cavity defects. As mentioned hereinabove, this can result in a leak of pressure or cooling medium gas from inside the compressor housing 1 to the outside.

In order to prevent the leak of pressure or cooling medium gas, the chill layer 2B in which no shrinkage cavity defects have appeared is formed to a thickness above a predetermined thickness at the casting surface, and when the cutting is performed with a predetermined cutting allowance, no shrinkage cavity defects are exposed on the cutting surface. Furthermore, locally cooling the cast holes with the core pins would be also effective for forming the chill layer 2B in which no shrinkage cavity defects have occurred to a thickness exceeding the cutting allowance. From among the core pins 5 and 6, the core pin 6 for the screw hole 3 has a small pin diameter, and providing a cooling medium flow channel inside thereof is difficult. For this reason, a flow channel for the cooling medium (water) is provided inside the core pin 5 with a comparatively large diameter that serves to mold the port hole 2, local cooling capacity with the core pin 5 is enhanced, and a region (chill layer 2B) where no shrinkage cavity defects occur is made thicker.

FIG. 4 shows a configuration of the core pin 5 provided with a flow channel for a cooling medium (water) inside thereof. The core pin 5 is a core pin 5 of a double pipe structure composed of a hollow pin body 5A, a holder 5C connected via a thread 5B to the upper portion of the pin body 5A, a plug 5D screwed into the end portion of the holder 5C, a central pipe 5E having one end thereof held in an up-down partition portion within the holder 5C and another end opened at the distant end portion inside the hollow pin body 5A, a cooling medium flow channel 5F formed between the hollow pin body 5A and the central pipe 5E and serving to pass the cooling medium (water) therethrough, a cooling medium supply pipe 5G connected to a space in the upper portion inside the holder 5C, and a cooling medium discharge pipe 5H connected to a space in the lower portion inside the holder 5C. The cooling medium (water) can flow at a preset flow rate from a water supply device 10 via the cooling medium supply pipe 5G and cooling medium discharge pipe 5H inside the core pin 5.

The core pin 5 can be replaced with a core pin 50 shown in FIG. 5. The core pin 50 has a partition plate structure in which the central pipe 5E of the core pin 5 is replaced with a partition plate 50E, one of the flow channels partitioned by the partition plate 50 is a cooling medium supply channel 50I and the other flow channel is a cooling medium discharge channel 50J. Other components are identical to those of the core pin 5 and assigned with identical symbols. The explanation thereof is omitted.

A method for forming the chill layer 2B with a thickness above a predetermined value in which no shrinkage cavity defects have occurred at the surface of the cast hole 2A serving as a rough hole for the port hole 2 by using the core pin 5 or 50 and a configuration of the compressor housing 1 provided with the chill layer 2B will be described below. First, the relationship between the temperature gradient and growth of dendrite arms during solidification shrinkage of the melt that is shown in FIG. 6 and FIG. 7 will be explained.
As shown in FIG. 6 and FIG. 7, the solidification of melt proceeds while the melt is supplied from a liquid phase side so as to compensate for the volume shrinkage that accompanies solidification between the dendrite arms 20 extending from the solid phase side. In order to prevent the occurrence of solidification shrinkage space (shrinkage cavity), it is necessary to supply a sufficient amount of melt between the dendrite arms 20. For this purpose, it is important to inhibit the growth of dendrite arms 20. In other words, where the dendrite arms 20 grow, a sufficient amount of melt cannot be supplied therebetween and a solidification shrinkage space X (see FIG. 6) that will become a shrinkage cavity appears between the dendrite arms.

The growth of dendrite arms 20 can be inhibited by increasing the cooling capacity of the die and increasing the temperature gradient G. The temperature gradient G can be represented by the following formula: $G = \left({T}_{L}-{T}_{S}\right) / L$

In this formula T_{L} stands for a liquidus temperature, T_{S} for a solidus temperature, and L for a length of dendrite arms 20.
Where the temperature gradient G is small (the case shown in FIG. 6), the dendrite arms 20 grow and the length L thereof increases to L1. On the other hand, by increasing the temperature gradient G (the case shown in FIG. 7), it is possible to inhibit the growth of dendrite arms 20 and make the length L thereof as short as L2 (L1 > L2).

Further, the spacing between the secondary dendrite arms 21 (dendrite arm spacing, referred to hereinbelow as "DAS") can be decreased by increasing the temperature gradient G. As shown in FIG. 8, the DAS can be easily checked by using an optical microscope after completion of solidification. The DAS is a distance between the centers of adjacent secondary dendrite arms and is taken as an average value of secondary dendrite arm spacing in a portion where four or more of secondary dendrite arms are arranged continuously side by side. More specifically, a portion where four or more of secondary dendrite arms are arranged continuously side by side is selected, a total of n (n is 4 or more) secondary dendrite arm spacings 1 are measured, and a value of 1/(n - 1) is found. The measurements are preformed in three or more places and an arithmetical average of the results is found.

The temperature gradient G can be increased by increasing the cooling capacity of the mold. Therefore, apparently the DAS can be decreased and the thickness of the region (chill layer 2B) where no shrinkage cavities have occurred can be increased by increasing the flow rate of the cooling medium that cools the mold, thereby raising the cooling rate of the mold, and inhibiting the growth of dendrite arms 20 during solidification. Accordingly, the following test was performed.

In the test, the core pin 5 shown in FIG. 4 was used, the cast holes 2A and 3A for the port hole 2 and screw hole 3 were die cast with the core pins 5 and 6 (see FIG. 3), while varying the flow rate V (cc/s) of the cooling medium (water), the DAS (µm) in a location at a predetermined depth from the casting surface (surface of cast product) was measured by a linear intercept method, and the thickness t (mm) of the region (chill layer 2B) without the shrinkage cavity defects was measured. The measurement results are shown in Table 1.

**[Table 1]**

| Sample No. | Cooling water flow rate (cc/s) | Secondary dendrite arm spacing [DAS] (µm) | | | Thickness of region without shrinkage cavities (mm) |
|---|---|---|---|---|---|
| | | Depth from casting surface: 0.25 mm | Depth from casting surface: 1.0 mm | Depth from casting surface: 2.0 mm | |
| a-1 | 0 | 5.8 | 9.3 | 9.7 | 0.34 |
| a-2 | 0 | 5.1 | 8.0 | 10.1 | 0.3 |
| b-1 | 1.6 | 4.7 | 9.4 | 11.5 | 0.42 |
| b-2 | 1.6 | 4.5 | 7.5 | 10.5 | 0.39 |
| c-1 | 12 | 4.1 | 7.7 | 8.8 | 1.1 |
| c-2 | 12 | 4.0 | 7.3 | 7.8 | 0.86 |
| c-3 | 12 | 4.0 | 7.5 | 7.6 | 0.99 |
| d-1 | 20.7 | 3.2 | 7.3 | 8.0 | 0.92 |
| d-2 | 20.7 | 3.3 | 6.6 | 7.4 | 1.36 |

The casting conditions in the above-described process were as follows: melt temperature 665°C, die temperature 200°C, injection rate 0.2 m/s (low rate) and 2.3 m/s (high rate). These casting conditions are identical to a melt temperature of 640-690°C and mold temperature of 150-300°C that are typical molding conditions for casting the aluminum die cast housing 1. As for the conditions relating to the flow of cooling medium (water), the flow of cooling medium (water) was initiated simultaneously with the completion of injection and the flow passage time was 3 sec.

The test results were analyzed and the relationship between the flow rate V (cc/s) of the cooling medium (water) and the thickness t (mm) of the region without shrinkage cavity defects was plotted as shown in FIG. 9. A thick solid line in FIG. 9 connects the minimum values of the thickness t (mm) of the region without shrinkage cavities obtained at each flow rate V (cc/s) of cooling water. These results also demonstrated that the thickness t (mm) of the region without shrinkage cavities can be obtained by increasing the flow rate V (cc/s) of cooling water flowing in the core pin 5, increasing the cooling capacity with the core pin 5, and increasing the temperature gradient G during solidification. In particular, it was confirmed that the thickness t (mm) of the region without shrinkage cavities can be increased to 0.8 mm or more by raising the flow rate V (cc/s) of cooling water to 12.0 cc/s or more.

Further, a graph representing the relationship between the depth d (mm) from the casting surface (surface of cast product) where shrinkage cavities are observed and DAS (µm) is shown in FIG. 10. The region shown by thick solid lines in FIG. 10 indicates a region in which the depth d (mm) from the casting surface (surface of cast product) where shrinkage cavities are observed, that is, the thickness of the region without shrinkage cavities assumes a minimum value (tₘᵢₙ) in the molded products obtained at various flow rates V (cc/s) of cooling water shown by broken lines. This region could be considered as a threshold (5.5-6.9 µm) of DAS at which shrinkage cavities were observed, and it was made clear that the condition for DAS at which no shrinkage cavities occur was 5.5 µm or less.

The above-described results demonstrated that by inhibiting the growth of dendrites during melt solidification shrinkage and making the DAS (secondary dendrite arm spacing) at least 5.5 µm or less, it is possible to form the chill layer 2B (see FIG. 2) in which shrinkage cavity defects causing pressure leak or gas leak in the compressor housing do not occur and which has a thickness equal to or larger than a predetermined thickness.

In the present embodiment, the chill layer 2B with a DAS of 5.5 µm or less was formed to a thickness more than a machining allowance in cutting after die casting at the surface of cast hole 2A for the port hole 2 cast with the core pin 5. Thus, in the case where the cutting allowance has a usual value of 0.5 mm, the chill layer 2B with a DAS of 5.5 µm or less was formed to a thickness of 0.5 mm or more, and the chill layer 2B with a DAS of 5.5 µm or less remained on the cut surface after cutting.

As a result, even when the cast hole 2A is used as a rough hole and subjected to cutting with the usual cutting allowance, no shrinkage cavity defects are exposed on the cut surface and the occurrence of pressure leak or gas leak via the cast hole 2A can be reliably prevented. Therefore, when the compressor housing 1 is manufactured, the production yield thereof can be greatly increased and the high-quality compressor housing 1 can be manufactured at a low cost.
In particular, by increasing the flow rate V (cc/s) of the cooling medium (water) flowing in the core pin 5 to 12.0 cc/s or more, it is possible to increase the thickness t (mm) of the region without shrinkage cavities in which DAS is 5.5 µm or less to be 0.8 (mm) or more and to eliminate reliably the occurrence of pressure leak or gas leak.

Further, in the above-described embodiment, the flow of the cooling medium in the core pins 5, 50 is initiated during die casting at the same time as the melt injection is completed, but performing the two actions simultaneously is not necessary. Thus, the cooling medium can be caused to flow immediately before the completion of melt injection, for example, from about 1 s before the completion of injection. In sum, where the cooling medium is left to flow or the cooling medium is caused to flow too early, the die is overcooled and an adverse effect is produced on the melt injection. Thus, part of the melt starts solidifying during loading or abnormal melt flow is induced. Therefore, the cooling medium may be caused to flow before the completion of injection, provided that no such adverse effect is produced.
Further, in the present embodiment, an example of applying the present invention to the compressor housing 1 is explained, but it goes without saying that the present invention is not limited to this application and can be applied to other pressure vessels.

## Claims

1. An aluminum die cast product comprising:
a cast hole (2A) formed in a thick portion (4) of the aluminum die cast product,
a chill layer (2B) on the surface of the cast hole (2A) with a thickness equal to, or larger than a predetermined thickness,
a secondary dendrite arm spacing (DAS) of 5.5 µm or less is provided at the cast hole (2A) in the chill layer (2B),
wherein the aluminum die cast product is a pressure vessel.

2. The aluminum die cast product according to claim 1, wherein
a thickness of the chill layer (2B) with a secondary dendrite arm spacing (DAS) of 5.5 µm or less is larger than a cutting allowance of the cast hole (2A) that is set in advance.

3. The aluminum die cast product according to claim 2, wherein
the chill layer (2B) with a secondary dendrite arm spacing (DAS) of 5.5 µm or less remains after cutting has been performed with the cutting allowance.

4. The aluminum die cast product according to any one of claims 1 to 3, wherein
a thickness of the chill layer (2B) is at least 0.5 mm or more.

5. The aluminum die cast product according to claim 1, wherein
the pressure vessel is a compressor housing (1).

6. A method for manufacturing an aluminum die cast product which is a pressure vessel having a thick portion (4) the method comprising:
forming a chill layer (2B) having a thickness equal to, or larger than a predetermined thickness
forming a cast hole (2A) by a core pin (5,50)in a thick portion (4) of the aluminum die cast product;
causing a secondary dendrite arm spacing (DAS) of 5.5 µm or less to form at a portion of the chill layer (2B) where the cast hole (2A) is formed in the thick portion (4) of die cast product by passing a flow of a cooling medium through the core pin (5, 50) and locally cooling the cast hole (2A).

7. The method for manufacturing an aluminum die cast product according to claim 6, wherein the method comprises:
using a core pin (5) with a double-pipe structure in which a central pipe is inserted into a hollow core pin body (5A),
supplying the cooling medium from the central pipe (5E) to a distal end portion of the core pin, the cooling medium being forced to flow into a cooling medium channel (5F) between the central pipe (5E) and the pin body (5A) to locally cool the cast hole.

8. The method for manufacturing an aluminum die cast product according to claim 7, wherein the method comprises:
causing the cooling medium to flow at a flow rate of 12 cc/s or more.

9. The method for manufacturing an aluminum die cast product according to claim 6, wherein method comprises:
inserting a core pin (50) of a partition plate structure in which a partition plate (50E) arranged along a pin axial direction into a hollow core pin body (5A);
supplying the cooling medium from one of the cooling medium channels (50I) partitioned by the partition plate; and
causing the cooling medium to flow into the other cooling medium channel (50J) to locally cool the cast hole.

10. The method for manufacturing an aluminum die cast product according to any one of claims 7 to 9, wherein initiating the flow of the cooling medium simultaneously with, or immediately prior to, the completion of a melt injection.

## Patentansprüche

1. Aluminiumdruckgußprodukt, umfassend:
eine gegossene Öffnung (2A), die in einem dicken Abschnitt (4) des Aluminiumdruckgußproduktes ausgebildet ist,
eine Schreckschicht (2B) auf der Oberfläche der gegossenen Öffnung (2A) mit einer Dicke, die gleich oder größer als eine vorbestimmte Dicke ist,
einen sekundären Dendritenarmabstand (DAS) von 5,5 µm oder weniger, der an der gegossenen Öffnung (2A) in der Schreckschicht (2B) vorgesehen ist, wobei das Aluminiumdruckgußprodukt ein Druckkessel ist.

2. Aluminiumdruckgußprodukt nach Anspruch 1, wobei
eine Dicke der Kühlschicht (2B) mit einem sekundären Dendritenarmabstand (DAS) von 5,5 µm oder weniger größer als eine voreingestellte Frästoleranz der gegossenen Öffnung (2A) ist.

3. Aluminiumdruckgußprodukt nach Anspruch 2, wobei
die Schreckschicht (2B) mit einem sekundären Dendritenarmabstand (DAS) von 5,5 µm oder weniger verbleibt, wenn mit der Frästoleranz gefräst wurde.

4. Aluminiumdruckgußprodukt nach einem der Ansprüche 1 bis 3, wobei eine Dicke der Schreckschicht (2B) wenigstens 0,5 mm oder mehr beträgt.

5. Aluminiumdruckgußprodukt nach Anspruch 1, wobei
der Druckkessel ein Kompressorgehäuse (1) ist.

6. Verfahren zum Herstellen eines Aluminiumdruckgußproduktes, das ein Druckkessel mit einem dicken Abschnitt (4) ist, wobei das Verfahren umfaßt:
Ausbilden einer Schreckschicht (2B) mit einer Dicke, die gleich oder größer als eine vorbestimmte Dicke ist,
Ausbilden einer gegossenen Öffnung (2A) durch einen Kernstift (5, 50) in einem dicken Abschnitt (4) des Aluminiumdruckgußproduktes,
Bewirken, daß sich ein sekundärer Dendritenarmabstand (DAS) von 5,5 µm oder weniger an einem Abschnitt der Schreckschicht (2B) bildet, wo die gegossene Öffnung (2A) in dem dicken Abschnitt (4) des Druckgußproduktes ausgebildet ist, durch Leiten eines Kühlflusses durch den Kernstift (5, 50) und lokales Kühlen der gegossenen Öffnung (2A).

7. Verfahren zum Herstellen eines Aluminiumdruckgußproduktes nach Anspruch 6, wobei das Verfahren umfaßt:
Verwenden eines Kernstiftes (5) mit einer Doppelrohrstruktur, in dem ein zentrales Rohr in einen Hohlkernstiftkörper (5A) eingeführt ist,
Zuführen des Kühlmediums aus dem zentralen Rohr (5E) zu einem distalen Endabschnitt des Kernstiftes, wobei das Kühlmedium gezwungen wird, in einem Kühlmediumkanal (5F) zwischen dem mittleren Rohr (5E) und dem Stiftkörper (5A) zu fließen, um die gegossene Öffnung lokal zu kühlen.

8. Verfahren zum Herstellen eines Aluminiumdruckgußproduktes nach Anspruch 7, wobei das Verfahren umfaßt:
Hervorrufen, daß das Kühlmedium mit einer Flußrate von 12 cc/s oder mehr fließt.

9. Verfahren zum Herstellen eines Aluminiumdruckgußproduktes nach Anspruch 6, wobei das Verfahren umfaßt:
Einführen eines Kernstiftes (50) einer Trennblechstruktur, in dem ein Trennblech (50E), das entlang einer axialen Stiftrichtung angeordnet ist, in einen Hohlkörperstiftkörper (5A) eingeführt ist,
Zuführen des Kühlmediums von einem der Kühlmediumkanäle (50I), die durch das Trennblech getrennt sind, und
Hervorrufen, daß das Kühlmedium in den anderen Kühlmediumkanal (50J) fließt, um die gegossene Öffnung lokal zu kühlen.

10. Verfahren zum Herstellen eines Aluminiumdruckgußproduktes nach einem der Ansprüche 7 bis 9, wobei Initiieren des Flusses des Kühlmediums gleichzeitig mit oder unmittelbar vor Vervollständigung einer Schmelzeneinspritzung erfolgt.

## Revendications

1. Produit de coulée sous pression d'aluminium comprenant :
un trou de coulée (2A) formé dans une partie épaisse (4) du produit de coulée sous pression d'aluminium,
une couche de refroidissement (2B) sur la surface du trou de coulée (2A) avec une épaisseur égale ou supérieure à une épaisseur prédéterminée,
un espacement des bras de dendrite (DAS) secondaires de 5,5 µm ou moins étant prévu au niveau du trou de coulée (2A) dans la couche de refroidissement (2B),
dans lequel le produit de coulée sous pression d'aluminium est un contenant sous pression.

2. Produit de coulée sous pression d'aluminium selon la revendication 1, dans lequel
une épaisseur de la couche de refroidissement (2B) avec un espacement des bras de dendrite (DAS) secondaires de 5,5 µm ou moins est supérieure à une tolérance d'usinage du trou de coulée (2A) qui est fixée à l'avance.

3. Produit de coulée sous pression d'aluminium selon la revendication 2, dans lequel
la couche de refroidissement (2B) avec un espacement des bras de dendrite (DAS) secondaires de 5,5 µm ou moins subsiste après qu'un usinage a été effectué avec la tolérance d'usinage.

4. Produit de coulée sous pression d'aluminium selon l'une quelconque des revendications 1 à 3, dans lequel
une épaisseur de la couche de refroidissement (2B) est d'au moins 0,5 mm ou plus.

5. Produit de coulée sous pression d'aluminium selon la revendication 1, dans lequel
le contenant sous pression est un logement de compresseur (1).

6. Procédé de fabrication d'un produit de coulée sous pression d'aluminium qui est un contenant sous pression ayant une partie épaisse (4), le procédé comprenant :
la formation d'une couche de refroidissement (2B) ayant une épaisseur égale ou supérieure à une épaisseur prédéterminée ;
la formation d'un trou de coulée (2A) par une broche-noyau (5, 50) dans une partie épaisse (4) du produit de coulée sous pression d'aluminium ;
la formation d'un espacement des bras de dendrite (DAS) secondaires de 5,5 µm ou moins au niveau d'une partie de la couche de refroidissement (2B) où le trou de coulée (2A) est formé dans la partie épaisse (4) du produit de coulée sous pression en faisant passer un flux d'un milieu de refroidissement à travers la broche-noyau (5, 50) et en refroidissant localement le trou de coulée (2A).

7. Procédé de fabrication d'un produit de coulée sous pression d'aluminium selon la revendication 6, dans lequel le procédé comprend :
l'utilisation d'une broche-noyau (5) avec une structure à deux tuyaux dans laquelle un tuyau central est inséré dans un corps de broche-noyau creux (5A),
la fourniture du milieu de refroidissement depuis le tuyau central (5E) jusqu'à une partie d'extrémité distale de la broche-noyau, le milieu de refroidissement étant forcé à s'écouler dans un canal de milieu de refroidissement (5F) entre le tuyau central (5E) et le corps de broche (5A) pour refroidir localement le trou de coulée.

8. Procédé de fabrication d'un produit de coulée sous pression d'aluminium selon la revendication 7, dans lequel le procédé comprend :
la mise en circulation du milieu de refroidissement à un débit de 12 cm³/s ou plus.

9. Procédé de fabrication d'un produit de coulée sous pression d'aluminium selon la revendication 6, dans lequel le procédé comprend :
l'insertion d'une broche-noyau (50) d'une structure de plaque de séparation dans laquelle une plaque de séparation (50E) est agencée le long d'une direction axiale de broche dans un corps de broche-noyau creux (5A) ;
la fourniture du milieu de refroidissement à partir de l'un des canaux de milieu de refroidissement (501) séparés par la plaque de séparation ; et
la mise en circulation du milieu de refroidissement dans l'autre canal de milieu de refroidissement (50J) pour refroidir localement le trou de coulée.

10. Procédé de fabrication d'un produit de coulée sous pression d'aluminium selon l'une quelconque des revendications 7 à 9, dans lequel la circulation du milieu de refroidissement est lancée simultanément avec, ou immédiatement avant, l'achèvement d'une injection de matière fondue.
